

## 1

3,034,957

SYNTHETIC FIBERS AND FABRICS HAVING  
MICROBICIDAL ACTIVITY

James L. Smith and Robert C. Harrington, Jr., Kingsport, Tenn., assignors to Eastman Kodak Company, Rochester, N.Y., a corporation of New Jersey  
No Drawing. Filed July 2, 1958, Ser. No. 746,076  
10 Claims. (Cl. 167—38.5)

This invention relates to improved fibers and fabrics, and more particularly, to synthetic fibers and fabrics of cellulose acetate, resins comprising copolymers of vinylidene chloride with acrylonitrile, and polyesters of 1,4-cyclohexanediethanol and terephthalic acid having microbicidal activity.

For many years, attempts have been made to produce fibers and fabrics which would effectively retard the growth of various microorganisms. Generally, this purpose has been accomplished by a separate treatment in which the fabric is coated with a resinous material containing a microbicide. Such a treatment has proved to be relatively ineffective because the resin coating would tend to flake off in normal use, and the usual washing or laundering operation would very quickly destroy whatever microbicidal properties that might be present. In addition, resinous coatings tend to change the hand of fabrics in an undesirable manner. Other treatments have consisted of treating the fabric in a solution of a microbicide. Fabrics containing some of these microbicidal agents are claimed to be substantive, but the microbicidal agents are actually held so loosely that they can be easily laundered out. Hence, it is desirable to have synthetic fibers and fabrics that have permanence of microbicidal activity, this result being obtained without affecting the appearance and physical properties thereof.

Also, any microbicidal additive to a fiber or fabric for clothing use, while it must be sufficient to kill or inhibit the growth of microorganisms, it must not be toxic or poisonous to the wearer of the clothing. In addition, any additive to a synthetic textile fiber must be compatible with the particular synthetic resin, have no adverse effects on dyeing characteristics and create no difficulty in the spinning thereof, many effective microbicides for a wide variety of substrates failing to meet these and the other above-described requirements in synthetic fibers and fabrics.

It is an object of this invention to provide novel synthetic fibers and fabrics having improved microbiological growth inhibition.

It is another object of this invention to provide novel synthetic fibers and fabrics capable of retaining microbiological growth inhibition properties after repeated washings or launderings, dry cleanings and wearings.

It is another object of this invention to provide novel synthetic fibers and fabrics having microbicidal activity which are not significantly different from corresponding fibers and fabrics without such activity with respect to hand, dyeability, appearance, and the like.

It is another object of this invention to provide novel synthetic fibers and fabrics capable of inhibiting microbiological growth and which are amenable to the various phases of fiber and fabric processing without loss of this inhibitory power.

It is still another object of this invention to provide novel synthetic fibers or fabrics prepared therefrom which will resist the formation of obnoxious odors after having become contaminated by perspiration or like soiling agents.

It is likewise an object of this invention to provide novel sanitary synthetic fibers or fabrics prepared therefrom such that microbiological contamination spread from

## 2

one wearer to another or from one place on a wearer's body to another would be significantly reduced or eliminated.

It is also an object of this invention to provide novel fibers and fabrics of cellulose acetate, resins comprising copolymers of vinylidene chloride and acrylonitrile, and polyesters of 1,4-cyclohexanediethanol and terephthalic acid having microbicidal activity.

These and other objects are attained by means of this invention as described hereinafter with reference to preferred embodiments thereof.

We have found that relatively low concentrations of 3,4,4'-trichlorocarbanilide can be incorporated into a solution or melt of cellulose acetate, resins comprising copolymers of vinylidene chloride and acrylonitrile or polyesters of 1,4-cyclohexanediethanol and terephthalic acid, and spun, extruded or drawn into fibers by conventional methods to produce improved fibers having microbicidal activity. By incorporating 3,4,4'-trichlorocarbanilide into the liquid resin prior to spinning, a fiber results which has the 3,4,4'-trichlorocarbanilide substantially uniformly distributed therein. Thus, fabrics prepared from such fibers have the 3,4,4'-trichlorocarbanilide microbicide built in or locked in. Thus, the synthetic fibers and fabrics of the invention are quite unlike natural and synthetic fibers and fabrics which have been superficially surface treated with various agents. The microbicide in the synthetic fibers and fabrics of the invention is available to render its microbicidal effect and yet can not be completely removed by repeated washings, dry cleanings and abrasions, such properties not being possessed by conventional surface treated fibers and fabrics.

The resins or plastic compositions comprising the fibers or fabrics of the invention are cellulose acetate, resins comprising copolymers of vinylidene chloride and acrylonitrile, and polyesters of 1,4-cyclohexanediethanol and terephthalic acid. Polyesters of 1,4-cyclohexanediethanol and terephthalic acid, and their method of preparation, are described in the copending application, Kibler et al., U.S. Serial No. 554,639, filed December 22, 1955, now U.S. Patent No. 2,901,466. Cellulose acetate is a well-known resin and can be prepared and spun into fibers by such methods as are disclosed in Stone U.S. Patent No. 2,000,047 and Stone U.S. Patent No. 2,000,048. Cellulose acetates having acetyl contents of about 38% to 45% by weight are suitable, with acetyl contents of about 38% to 41% being preferred. Fiber-forming resins comprising copolymers of vinylidene chloride and acrylonitrile are also known in the art, such being disclosed in Coover et al. U.S. Patent No. 2,831,826. Preferred fiber-forming resins of this latter type are mixtures comprising (A) 70% to 95% by weight of a copolymer of from 30% to 65% by weight of vinylidene chloride and 70% to 35% by weight of acrylonitrile, and (B) 30% to 5% by weight of a second polymer consisting of (1) a homopolymer of an N-alkyl acrylamide where the alkyl group contains 1 to 6 carbon atoms, or (2) a copolymer of an N-alkyl acrylamide and an N-alkyl methacrylamide wherein the alkyl group contains 1 to 6 carbon atoms, or (3) a copolymer consisting of at least 50% by weight of an N-alkyl acrylamide wherein the alkyl group contains 1 to 6 carbon atoms and not more than 50% by weight of a polymerizable monovinyl pyridine monomer. The second polymeric material added to the copolymer of vinylidene chloride and acrylonitrile is added mainly to improve the dyeing characteristics of the composition and typically includes such materials as poly-N-isopropyl acrylamides, a copolymer of N-isopropyl acrylamide and 2-methyl-5-vinyl pyridine, a copolymer of N-tert-butyl acrylamide and 2-methyl-5-vinyl pyridine, a copolymer of N-isopropyl acrylamide and N-methyl methacrylamide, or related polymeric materials. The

preparation of such mixtures is described in detail in the aforementioned Coover et al. patent.

The microbicide employed in the synthetic fibers and fabrics of the invention, 3,4,4'-trichlorocarbanilide, can be readily prepared by refluxing equal molar proportions of 3,4-dichloroaniline and 4-chlorophenyl isocyanate in an inert solvent such as diethyl ether. This microbicide is incorporated into a solution or dope or melt of the resin and thereafter spun by conventional methods into textile fibers to contain about .05% to 5%, and preferably .2% to 2%, by weight of the microbicide based on the weight of the synthetic fiber. The microbicide is substantially uniformly distributed in the fiber. Such fibers can thereafter be woven into fabrics, or they can be combined with other fibers, natural or synthetic, and woven into fabrics. These fibers and fabrics have substantial microboidal activity against such microorganisms as *Micrococcus pyogenes* var. *aureus*, *Micrococcus epidermidis*, *Micrococcus pyogenes*, *Diplococcus pneumoniae*, *Corynebacterium diphtheriae*, *Streptococcus viridans*, *Lactobacillus casei*, and related microorganisms. The synthetic fibers and fabrics of the invention show particular microboidal activity toward gram positive microorganisms. However, while the fibers and fabrics of the invention have microboidal activity, they are substantially non-toxic and non-irritating to humans and thus can be used in clothing, blankets, carpeting, and for numerous other uses.

A particularly desirable property of the present fibers and fabrics is the permanence of the 3,4,4'-trichlorocarbanilide distributed therein. Even in view of the substantial surface area of fabrics prepared from the present synthetic fibers, these fabrics can be subjected to more than 25 washings in household washing machines in the usual manner and still exhibit microboidal activity. Likewise, this microboidal activity can not be lost by mechanical abrasion of the fibers or the fabrics of the invention such as normally results in the processing and use thereof. This permanence of microboidal activity is attributed to the incorporation of the 3,4,4'-trichlorocarbanilide in the dope or melt of the resin before spinning into fibers as distinguished from coating the finished fabric with a microboidal material.

The addition of 3,4,4'-trichlorocarbanilide in the above-defined amounts does not adversely affect the physical properties of the fibers and fabrics of the invention such as strength, elongation, hand and luster. In addition, this microbicide is compatible in the fibers and fabrics of the invention as it does not oil out and does not cause discolorating thereof under usual processing and usage. Also, this microbicide creates no difficulty in the spinning of the fiber or in the dyeing of the fiber or fabric.

The invention is further illustrated by the following examples of preferred embodiments thereof.

#### Example 1

A cellulose acetate dope in acetone containing 28.5% by weight of cellulose acetate having an acetyl content of about 39% was prepared. To the dope was added 1% by weight of 3,4,4'-trichlorocarbanilide based on the weight of the cellulose acetate. The resulting mixture was blended and thereafter spun from the acetone into 55 denier, 13 filament fibers. The resulting fibers containing about 1% by weight of 3,4,4'-trichlorocarbanilide substantially uniformly distributed therein were then woven into a fabric in the usual manner. The prepared fabric showed inhibition against *Micrococcus pyogenes* var. *aureus* after 25 launderings in the usual manner in a conventional household washing machine. This inhibition was determined by placing samples of the fabric in a petri dish containing nutrient agar surface inoculated with the microorganism, a clear zone being formed around the test samples. The prepared fabric has similar permanence of microboidal resistance to *Micrococcus epidermidis*, *Micrococcus pyogenes*, *Diplococcus pneumoniae*, *Corynebacterium diphtheriae* and *Streptococcus*

*viridans*. Similar results were obtained with fabrics prepared from cellulose acetate fibers containing 0.3% and 1.5% by weight of 3,4,4'-trichlorocarbanilide. The described cellulose acetate fabrics containing the 3,4,4'-trichlorocarbanilide did not differ noticeably in dyeability, hand and physical appearance from comparable cellulose acetate fabrics containing no 3,4,4'-trichlorocarbanilide.

#### Example 2

10 A copolymer prepared from about 50% by weight of vinylidene chloride and 50% by weight of acrylonitrile was prepared in accordance with the method described in Example 1 of Coover et al. U.S. Patent No. 2,831,826 and thereafter dissolved in about four times its weight of dimethyl formamide. Then sufficient 3,4,4'-trichlorocarbanilide was added to the resulting dope which was spun into fibers as described in Example 1 above to produce fibers having about 1% by weight of the 3,4,4'-trichlorocarbanilide substantially uniformly distributed therein. Fabrics prepared from the resulting fibers have permanence of microboidal activity after more than 25 washings as described in Example 1 above. The described microboidal fabric does not differ noticeably in dyeability, hand and physical appearance from comparable fabrics containing no 3,4,4'-trichlorocarbanilide.

#### Example 3

Several fiber-forming mixtures of polymers prepared in accordance with the method of Coover et al. U.S. Patent No. 2,831,826, were spun from acetone and woven into fabrics as described in Example 1 above. With 1% by weight of 3,4,4'-trichlorocarbanilide substantially uniformly dispersed in the prepared fiber-forming polymers, the fabrics prepared therefrom have substantial microboidal activity. The prepared fibers had the following compositions: (a) a mixture of 85% by weight of a copolymer of 52% by weight of acrylonitrile and 48% vinylidene chloride, and 15% by weight of poly-N-isopropyl acrylamide; (b) a mixture of 70% by weight of a copolymer of 50% by weight of acrylonitrile and 50% by weight of vinylidene chloride, and 30% by weight of a copolymer of 90% by weight of N-tert. butyl acrylamide and 10% by weight of 2-methyl-5-vinyl pyridine; (c) a mixture of 90% by weight of a copolymer of 50% by weight of acrylonitrile and 50% by weight of vinylidene chloride, and 10% by weight of a copolymer of N-isopropyl acrylamide and 2-methyl-5-vinyl pyridine; and, (d) a mixture of 70% by weight of a copolymer of 50% by weight of acrylonitrile and 50% by weight of vinylidene chloride, and 30% by weight of a copolymer of 90% by weight of N-isopropyl acrylamide and 10% by weight of N-methyl methacrylamide. Fabrics prepared from these fibers show permanence of microboidal activity when tested as described in Example 1 above. The described synthetic fabrics do not differ noticeably in dyeability, hand and physical appearance from comparable fabrics containing no 3,4,4'-trichlorocarbanilide.

#### Example 4

60 A polyester of 1,4-cyclohexanedimethanol and terephthalic acid was prepared by reacting 1,4-cyclohexanedimethanol (70% trans, 30% cis) and dimethyl terephthalate in accordance with the method described in Example 1 of copending Kibler et al. application, U. S. Serial No. 554,639, filed December 22, 1955. By drawing a melt 65 of the resulting polymer containing 1% by weight of 3,4,4'-trichlorocarbanilide into fibers, and spinning the fibers into a fabric, a fabric results that has substantial microboidal activity. Such a fabric has permanence of microboidal activity after more than 25 washings as described in Example 1 above. The described microboidal fabric does not differ noticeably in dyeability, hand and physical appearance from comparable fabrics containing no 3,4,4'-trichlorocarbanilide.

70 The microbicide of the invention can be prepared by the method described in Example 5 below.

## Example 5

To a suitable reaction vessel equipped with a thermometer, agitator and reflux condenser and containing 8.1 parts by weight of 3,4-dichloroaniline in 57 parts by weight of diethyl ether is added dropwise a solution of 7.7 parts by weight of 4-chlorophenyl isocyanate in 15 parts by weight of diethyl ether at such a rate as to maintain gentle reflux. Upon completion of the isocyanate addition the reaction mass is agitated for about one hour. The mass is filtered and the residue washed with diethyl ether. The resulting 3,4,4'-trichlorocarbanilide product can be further purified by recrystallization from ethanol.

The present invention thus provides novel synthetic textile fibers and fabrics which have considerable utility because of their built in or locked in microbicidal activity, this microbicidal activity having a permanence in the present fibers and fabrics not possessed by conventional surface treated fibers and fabrics. In addition the 3,4,4'-trichlorocarbanilide additive of the invention does not adversely affect the processing, physical appearance and physical properties of the subject fibers and fabrics.

Although the invention has been described in detail with reference to certain preferred embodiments thereof, it will be understood that variations and modifications can be effected within the spirit and scope of the invention as described hereinabove and as defined in the appended claims.

We claim:

1. A synthetic textile fiber having microbicidal activity having substantially uniformly dispersed therein .05% to 5% by weight of 3,4,4'-trichlorocarbanilide, said fiber comprising a resin from the group consisting of:

- (I) cellulose acetate having an acetyl content of about 38% to 45%;
- (II) a polyester comprised principally of the recurring structural unit



and;

- (III) a mixture of
  - (A) 70% to 95% by weight of a copolymer of 30% to 65% by weight of vinylidene chloride and 70% to 35% by weight of acrylonitrile, and
  - (B) 30% to 5% by weight of a second polymer from the group consisting of
    - (1) a homopolymer of N-alkyl acrylamide wherein the alkyl group contains 1 to 6 carbon atoms,
    - (2) a copolymer of N-alkyl acrylamide and N-alkyl methacrylamide wherein the alkyl group contains 1 to 6 carbon atoms, and
    - (3) a copolymer consisting of at least 50% by weight of an N-alkyl acrylamide wherein the alkyl group contains 1 to 6 carbon atoms and not more than 50% by weight of a polymerizable monovinyl pyridine monomer.

2. A synthetic textile fiber having microbicidal activity comprising cellulose acetate having an acetyl content of about 38% to 45% with .2% to 2% by weight of 3,4,4'-trichlorocarbanilide substantially uniformly distributed therein.

3. A synthetic textile fiber having microbicidal activity comprising cellulose acetate having an acetyl content of about 38% to 41% with .2% to 2% by weight of 3,4,4'-trichlorocarbanilide substantially uniformly dispersed therein.

4. A synthetic textile fiber having microbicidal activity comprising a mixture of (A) 70% to 95% by weight of

a copolymer of from 30% to 65% by weight of vinylidene chloride and 70% to 35% by weight of acrylonitrile, and (B) 30% to 5% by weight of a second polymer from the group consisting of (1) a homopolymer of an N-alkyl acrylamide wherein the alkyl group contains 1 to 6 carbon atoms, (2) a copolymer of an N-alkyl acrylamide and N-alkyl methacrylamide wherein in the alkyl group contains 1 to 6 carbon atoms, and (3) a copolymer consisting of at least 50% by weight of an N-alkyl acrylamide wherein the alkyl group contains 1 to 6 carbon atoms and not more than 50% by weight of a polymerizable monovinyl pyridine monomer, with .2% to 2% by weight of 3,4,4'-trichlorocarbanilide substantially uniformly distributed therein.

5. A synthetic textile fiber having microbicidal activity comprising a mixture of (A) 70% to 95% by weight of a copolymer of from 30% to 65% by weight of vinylidene chloride and 70% to 35% by weight of acrylonitrile, and (B) 30% to 5% by weight of poly-N-isopropylacrylamide, with .2% to 2% by weight of 3,4,4'-trichlorocarbanilide substantially uniformly distributed therein.

6. A synthetic textile fiber having microbicidal activity comprising a mixture of (A) 70% to 95% by weight of a copolymer of from 30% to 65% by weight of vinylidene chloride and 70% to 35% by weight of acrylonitrile, and (B) 30% to 5% by weight of a copolymer of N-isopropyl acrylamide and 2-methyl-5-vinyl pyridine, with .2% to 2% by weight of 3,4,4'-trichlorocarbanilide substantially uniformly distributed therein.

7. A synthetic textile fiber having microbicidal activity comprising a mixture of (A) 70% to 95% by weight of a copolymer of from 30% to 65% by weight of vinylidene chloride and 70% to 35% by weight of acrylonitrile, and (B) 30% to 5% by weight of a copolymer consisting of at least 50% by weight of N-isopropyl acrylamide and not more than 50% by weight of N-methyl methacrylamide, with .2% to 2% by weight of 3,4,4'-trichlorocarbanilide substantially uniformly distributed therein.

8. A synthetic textile fiber having microbicidal activity comprising a mixture of (A) 70% to 95% by weight of a copolymer of from 30% to 65% by weight of vinylidene chloride and 70% to 35% by weight of acrylonitrile, and (B) 30% to 5% by weight of a copolymer of N-tert. butyl acrylamide and 2-methyl-5-vinyl pyridine, with .2% to 2% by weight of 3,4,4'-trichlorocarbanilide substantially uniformly distributed therein.

9. A synthetic textile fiber having microbicidal activity comprising a polyester of 1,4-cyclohexanedimethanol and terephthalic acid having the recurring structural unit



55 with .2% to 2% by weight of 3,4,4'-trichlorocarbanilide substantially uniformly dispersed therein.

10. A fabric having microbiological activity comprising fibers as defined in claim 1.

## 60 References Cited in the file of this patent

## UNITED STATES PATENTS

|           |               |       |               |
|-----------|---------------|-------|---------------|
| 2,695,858 | Lisle         | ----- | Nov. 30, 1954 |
| 2,758,955 | Johnson       | ----- | Aug. 14, 1956 |
| 2,774,708 | Cohen         | ----- | Dec. 18, 1956 |
| 2,812,332 | Pennino       | ----- | Nov. 5, 1957  |
| 2,846,398 | Beaver et al. | ----- | Aug. 5, 1958  |
| 2,913,369 | Haslam        | ----- | Nov. 17, 1959 |

## 70 FOREIGN PATENTS

|         |               |       |               |
|---------|---------------|-------|---------------|
| 627,710 | Great Britain | ----- | Aug. 15, 1949 |
| 684,404 | Great Britain | ----- | Dec. 17, 1952 |
| 709,982 | Great Britain | ----- | June 2, 1954  |

UNITED STATES PATENT OFFICE  
CERTIFICATION OF CORRECTION

Patent No. 3,034,957

May 15, 1962

James L. Smith et al.

It is hereby certified that error appears in the above numbered patent requiring correction and that the said Letters Patent should read as corrected below.

Column 4, line 70, for "ni" read -- in --; column 5, lines 39 to 42, the formula should appear as shown below instead of as in the patent:



Signed and sealed this 16th day of October 1962.

(SEAL)

Attest:

ERNEST W. SWIDER

Attesting Officer

DAVID L. LADD

Commissioner of Patents